

# United States Patent

[11] 3,617,267

[72] Inventor William C. Kinney  
Littleton, Mass.  
[21] Appl. No. 819,075  
[22] Filed Apr. 24, 1969  
[45] Patented Nov. 2, 1971  
[73] Assignee Itek Corporation  
Lexington, Mass.

3,382,068 5/1968 Gold..... 96/27  
3,429,706 2/1967 Shepard et al. .... 96/1 X

Primary Examiner—George F. Lesmes  
Assistant Examiner—M. B. Wittenberg  
Attorneys—Homer O. Blair, Robert L. Nathans, W. Gary  
Goodson and David E. Brook

[54] **PROCESS FOR FORMING A SERIES OF MASTERS IN REGISTER**  
16 Claims, 3 Drawing Figs.

[52] U.S. Cl..... 96/1, 96/41,  
96/27, 96/1.5, 101/456  
[51] Int. Cl..... G03g 5/00,  
G03c 5/04  
[50] Field of Search..... 96/41, 44,  
67, 75, 1, 1.5, 12

[56] **References Cited**

UNITED STATES PATENTS

2,814,565 11/1957 Long ..... 96/12  
3,157,499 11/1964 Trusheim ..... 96/67

**ABSTRACT:** A process is disclosed for forming a series of masters which reproduce in register selected portions of an original by using a plurality of photosensitive scribable copy media which can be updated. A visible image of the original is formed on each piece of photosensitive scribable copy medium and then an area of the scribable coating is scribed on one of the media corresponding to a selected portion of the original for which a separate master is to be formed. A visible image of the previously scribed area is then formed on another copy medium thereby updating said copy medium. If more than two masters are to be formed, the scribing and updating steps are repeated for each additional portion of the original for which a separate master is to be formed, except for the last of these portions. For the last portion, only the scribing step is repeated.



PATENTED NOV 2 1971

3,617,267



FIG. I.

FIG. II.

FIG. III.



WILLIAM C. KINNEY  
INVENTOR

BY *David E. Brook*

ATTORNEY.

PROCESS FOR FORMING A SERIES OF MASTERS IN  
REGISTER

BACKGROUND OF THE INVENTION

1. Field of the Invention

This invention relates to a process for using scribable copy media and more particularly to a process for using photosensitive scribble copy media capable of being updated to produce a series of masters which reproduce in register selected portions of an original.

2. Description of the Prior Art

Heretofore, there have been two methods for using photosensitive scribble copy media. In the first, the medium is scribed at selected areas and then used as a template. See Beeber et al., U.S. Pat. No. 2,999,016. In the second, the medium is selectively scribed down to a second intermediate photosensitive layer positioned between the base and scribble coating, exposed, and then color developed so that the scribed medium itself can be used as a master. See Trusheim, U.S. Pat. No. 3,157,499.

Neither of these previously known methods for using photosensitive scribble copy media are suitable for forming a series of masters which reproduce selected portions of an original so that the reproduced portions are in perfect register with each other.

SUMMARY OF THE INVENTION

The invention is a process for forming a series of masters which reproduce in register selected portions of an original. A plurality of photosensitive scribble copy media capable of being updated are used in this process.

A visible image of the original is formed on each of the plurality of photosensitive scribble copy media. One of the media is then scribed at areas corresponding to a selected portion of the original for which a separate master is to be formed.

Another piece of the photosensitive scribble copy medium having a visible image of the original thereon is updated by the addition of a visible image of all previously scribed areas. Thus, any error in the previous scribings can be compensated for or any subsequent scribbling errors can be prevented when the updated copy medium is scribed so that perfect register between the various portions of the original will be preserved in reproductions because of the corrected masters.

The steps of scribing and updating the next copy medium to be scribed are repeated for each additional portion of the original for which a separate master is to be formed with the exception of the last portion. Only the scribing step is repeated for the last portion of the original for which a master is to be formed.

Masters can be formed from each scribed copy medium anytime subsequent to the scribing.

Although this process has many applications, it is particularly adapted to the field of colored mapmaking. In making copies of colored maps, it is customary to use a series of color separation printing plates to reproduce selected portions of the map. For example, one plate might reproduce the primary roads of a specific local which are to be red on the map, and another plate might reproduce the secondary roads of the same local which are to be blue on the map. Obviously each of the reproduced portions has to be in register with the other portions for mapmaking applications.

The claimed process allows the scribe to obtain perfect register between the reproduced portions even though one of the scribble copy media has been scribed out of registration. In other words, the claimed process allows the scribe to compensate for a registration error in scribing a prior copy medium because he can update all subsequent copy media before he actually scribes them. The updated copy media will show any errors in register due to the previous scribings, and the scribe simply takes these into account when he scribes the updated copy medium. Since the masters are formed from copy media which have been updated prior to being scribed,

the masters will reproduce each selected portion of the original with perfect register.

BRIEF DESCRIPTION OF THE DRAWINGS

5 FIG. 1 is a front view of an original which consists of a triangle, circle and square.

FIG. II is a perspective view of a photosensitive scribble copy medium capable of being updated.

10 FIG. III is a schematic diagram of a process for producing three masters which will reproduce the triangle, circle and square of the original in register.

DESCRIPTION OF THE PREFERRED EMBODIMENTS

15 The process of this invention is used to produce a series of masters, which will reproduce in register selected portions of an original. A composite reproduction of the original can be made by using each master in the series to reproduce its selected portion of the original.

20 For exact reproduction of the original, it is imperative that each reproduced portion be in register with all of the other reproduced portions. By "in register" is meant that the true alignment of portions of the original is maintained between those portions reproduced by the masters of this invention.

25 A plurality of photosensitive scribble copy media are used in the process of this invention. The specific number depends, of course, upon the number of selected portions of the original which are to be placed upon separate masters.

30 To be suitable for use with this invention, the photosensitive scribble copy media have to possess the capability to be updated. By "updating" is meant the addition of further data to a delineated area of a copy medium already carrying data. More specifically for purposes of this invention, updating can be

35 considered to be the addition of a visible image upon another visible image previously placed on a copy medium. Usually, updating involves the desensitization of photosensitive material containing one visible image and the exposing and developing to form a second visible image on the photosensitive 40 material. One such procedure suitable for updating copy media useful for this invention is described in more detail in Pfluke, U.S. Ser. No. 803,152, filed Feb. 2, 1969.

One copy medium having the capability of being updated is illustrated in FIG. II. A base 7 has a scribble coating 6 and a

45 photosensitive photoconductor 5 which is capable of being reversibly activated by activating radiation. Preferred photoconductors for use in this copy medium are compounds of a metal with a nonmetallic element of Group VIA of the periodic chart such as titanium dioxide. That titanium dioxide which has an average particle size of below about 250 millimicrons and which has been pretreated by maintaining it at a temperature of at least about 200° C. for a period of at least about one-half hour in the presence of an oxidizing atmosphere is particularly preferred because of the excellent results obtained with such titanium dioxide. A more detailed description of this photosensitive scribble copy medium capable of being updated is presented in Berman, U.S. Ser. No. 812,191, filed Apr. 1, 1969.

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 91

the photoconductor to an image and developing a visible image are well known by those skilled in the art. Examples of suitable techniques are described in U.S. Pat. Nos. 3,152,903 5 3,380,823 and 3,382,068. The visible image of the original is represented in FIG. III by the light lines shown on each of the photosensitive scribable copy media 9 and 10.

The scribable coating on one of the scribable copy media is scribed at areas corresponding to a selected portion of the original for which a separate master is to be formed. As shown by the dark solid line 12, an area corresponding to the square 10 2 is scribed on photosensitive scribable copy medium 8. Scribing can be accomplished by any standard means including heat, chemicals or the use of an instrument such as scribing tool commonly used by draftsmen.

Subsequently, a master 58 is formed using the scribed copy medium 8 which will reproduce the square 2.

The term "master" is used to mean any article which can be formed from the scribed copy medium and which will reproduce one or more copies of a selected portion of the original. It includes but is not limited to printing plates such as lithographic printing plates which have an oleophilic-hydrophilic differentiation and a printing plate containing diazo materials. The masters of this invention are formed by techniques well known to those skilled in the art and they can be formed immediately after each copy medium is scribed as illustrated in FIG. III or at any later time.

A visible image of each of the previously scribed areas of the photosensitive scribable copy media are now formed on another of the copy media. This updates the visible image of the original initially placed on the photosensitive scribable copy medium because the scribe can now see any misregistration caused by scribing the various areas on preceding copy media. If a registration error has been made, the scribe can compensate for the error when he scribes the next area so that perfect relative alignment will be maintained in the reproductions.

The updating feature can be further illustrated by use of FIG. III. Before or after the master 58 has been formed, the scribed area 12 of copy medium 8 is used to form a visible image of the scribed area 12 on the medium 9. The updating is indicated by the broken line 32 in the shape of a square on copy medium 9. If an error had been made in scribing the square 12, the updated square 32 would not coincide perfectly with the square portion of the visible image of the original initially placed upon photosensitive scribable copy medium 9. For example, if the area 12 had been scribed slightly to the left of its proper location, the updated square 32 would appear slightly to the left of the square portion of the original initially placed on the copy medium 9 and the scribe could take this into account by scribing the area 13 slightly to the left thereby preserving the relative alignment between the square and circle in reproductions made from masters 58 and 59.

Masters can be formed by passing activating radiation through the scribed areas of the photosensitive scribable copy media onto master material to form a latent image of the scribed areas and thereafter using standard master preparation techniques which are known to those skilled in the art. The term activating radiation includes visible light, electron beams and other forms of electromagnetic radiation capable of activating a photosensitive material. Contact printing or other similar techniques known to those skilled in the art can be used to update subsequent copy media with previously scribed areas.

Thereafter, the scribing and updating steps are performed for each remaining portion of the original for which a separate master is to be formed except the last portion. In FIG. III, the area 13 is scribed on the photosensitive scribable copy medium 9, the master 59 is formed to reproduce the circle 23 which corresponds to the scribed area 13, and the next photosensitive scribable copy medium 10 is updated by forming visible images of both the scribed area 12 and the scribed area 13 on the photosensitive scribable copy medium 10. The updating is indicated by the broken lines 33 and 42.

For the last portion of the original 1 for which a separate master is to be formed, the scribing step is repeated. As shown, the area 14 is scribed in the copy medium 10 and the master 60 is formed to reproduce the triangle 24 which corresponds to the scribed area 14 and the original tangle 4.

By this process, a series of masters 58, 59 and 60 are produced which each reproduce a predetermined portion of the original 1. Since the scribe is able to compensate for errors made in scribing any previous areas and to prevent errors in subsequently scribed areas the masters will reproduce the original in register.

If it is desired to reproduce the original so that each portion has a different color, this can be easily accomplished with the masters formed by this process. Assume, for example, that it is 15 desired to reproduce the original 1 so that the square is red, the circle is blue and the triangle is green. All that is required is to ink the master 58 with red ink, the master 59 with blue 20 ink and the master 60 with green ink. These masters will then 25 reproduce copies of the original with a red square, a blue circle and a green triangle, and the relative alignment between each portion of the original will be maintained in the reproductions regardless of errors made in scribing the areas 2 or 13 because such errors are compensated for in scribing subsequent portions.

As is apparent from the above description, the process of this invention is useful for forming masters from which 30 reproductions can be made. This process is particularly useful for any application in which it is desired to selectively place portions of an original on separate masters. It is especially applicable where each portion of the original is to be reproduced in a different color and where it is important to maintain the alignment of the portions, as for example, in the art of map-making.

The following example illustrates the invention. All parts and percentages are by weight unless otherwise specified.

#### EXAMPLE I

40 Six pounds of a homogenous dispersion of titanium dioxide in polyvinyl alcohol per 3,300 square feet are coated onto the surface of Keuffel and Esser scribable material, stock No. 44-3227, white with a red undercoat, and cured for 2½ minutes at 350° F. The pigment/binder ratio in the dispersion 45 is 1:1 and the titanium dioxide has an average particle size of less than 250 millimicrons.

The coated scribable copy medium is then exposed once at an instrument setting of  $10^{12}$  seconds using an EG&G Mark VI Sensitometer.

50 After exposure, the photosensitive scribable copy medium is placed in a beaker of 2.5N silver nitrate at 70° F. for 30 seconds with gentle agitation. Excess silver nitrate solution is removed with an air knife and the scribable copy medium is dried with hot air.

55 A developer solution having a pH of 3.5 and having the following ingredients is used:

|                              |         |
|------------------------------|---------|
| Metol                        | 34.0 g. |
| Diethylaminoethanethiol HCl  | 1.0 g.  |
| Sodium Thioglycolate         | 0.25 g. |
| Potassium hydrogen phthalate | 20.0 g. |
| Citric acid                  | 3.0 g.  |
| Water to 1.0 liter.          |         |

65 The exposed and sensitized photosensitive scribable copy medium is placed in a covered container of the developer solution at 70° F., and after waiting 5 seconds, the container is rapidly shaken for 25 seconds. After removal from the developer solution, the material is washed with water at 70° F. 70 for 3 minutes and dried with hot air.

A visible image having excellent overall quality is formed on the surface of the scribable material.

The same medium is updated by twice exposing it to an image pattern of activating radiation with the EG&G Mark VI 75 Sensitometer set at  $2 \times 10^{13}$  seconds and processing it in the

same manner as following initial exposure. Following this, the medium is immersed in Kodak F-5 fixing solution for 30 seconds at 70° F., washed with water, and dried with hot air. A second visible image having excellent overall quality now appears superimposed on the first image.

Further updating can be accomplished prior to fixing if desired.

What is claimed is:

1. A process for forming a series of masters which reproduce in register selected portions of an original using a plurality of photoconductive photosensitive scribble copy media which can be updated, comprising:
  - a. forming a visible image of the original on the plurality of photoconductive photosensitive scribble copy media;
  - b. scribing a first area of the visible image of the original on one of said media to form a first scribed area on the copy medium corresponding to a selected portion of the original for which a master is to be formed;
  - c. forming a visible image of the first area of said photoconductive photosensitive scribble copy medium scribed in step (b) upon another of the copy media which already has thereon a visible image of original whereby an error made in scribing said first area can be noted and compensated for in the scribing of a second area corresponding to another selected portion of the original on a second copy medium; and;
  - d. scribing said second area of the visible image of the original on said second copy medium.
2. A process of claim 1 wherein each of said photosensitive scribble copy media comprises a base with a scribble coating and a photosensitive photoconductor thereon, said photoconductor being reversibly activated when exposed to activating radiation.
3. A process of claim 2 wherein said photosensitive photoconductor comprises a compound of a metal with a non-metallic element of Group VIA of the periodic chart of the elements.
4. A process of claim 3 wherein said photosensitive photoconductor comprises titanium dioxide.
5. A process of claim 4 wherein said titanium dioxide has an average particle size of below about 250 millimicrons.
6. A process of claim 5 wherein said titanium dioxide has been pretreated by maintaining it at a temperature of at least about 200° C. for a period of at least about one-half hour in the presence of an oxidizing atmosphere.
7. A process of claim 6 wherein step (c) is accomplished by contact printing a visible image of the scribed area onto another photosensitive scribble copy medium which already

has thereon a visible image of the original.

8. A process for forming a series of masters which reproduce in register selected portions of an original using a plurality of photoconductive photosensitive scribble copy media which can be updated, comprising:

- a. forming a visible image of the original on the plurality of photoconductive photosensitive scribble copy media;
- b. scribing an area of the visible image of the original on one of said copy media to form a scribed area on the copy medium corresponding to a selected portion of the original for which a master is to be formed;
- c. forming a visible image of each area previously scribed in step (b) upon another of the copy media which already has thereon a visible image of the original whereby any errors made in scribing previous areas can be compensated for in scribing subsequent areas;
- d. thereafter repeating steps (b) and (c) for all but the last of the remaining selected portions of the original for which a master is to be formed; and,
- e. thereafter repeating only step (b) for the last selected portion of the original for which a master is to be formed.

9. A process of claim 8 wherein each of said photosensitive scribble copy media comprises a base with a scribble coating and a photosensitive photoconductor thereon, said photoconductor being reversibly activated when exposed to activating radiation.

10. A process of claim 9 wherein said photosensitive photoconductor is a compound of a metal with a nonmetallic element of Group VIA of the periodic chart of the elements.

11. A process of claim 10 wherein said photosensitive photoconductor comprises titanium dioxide.

12. A process of claim 11 wherein said titanium dioxide has an average particle size of below about 250 millimicrons.

13. A process of claim 12 wherein said titanium dioxide has been pretreated by maintaining it at a temperature of at least about 20° C. for a period of at least about one-half hour in the presence of an oxidizing atmosphere.

14. A process of claim 13 wherein step (c) is accomplished contact printing a visible image of the previously scribed areas onto another photosensitive scribble copy medium which already has thereon a visible image of the original.

15. A process of claim 3 including the additional step of forming a separate master from each of said scribed copy media.

16. A process of claim 9 including the additional step of forming a separate master from each of said scribed copy media.

\* \* \* \* \*